

## UNITED STATES PATENT OFFICE.

JACOB DOLFEN, OF BERN, SWITZERLAND, ASSIGNOR TO FRITZ HOSTETTLER, OF BERN, SWITZERLAND.

## MANUFACTURE OF LIQUID FUEL.

No Drawing.

Application filed January 18, 1922. Serial No. 530,191.

*To all whom it may concern:*

Be it known that I, JACOB DOLFEN, a citizen of the German Empire, residing at Bern, Switzerland, have invented certain new and useful Improvements in the Manufacture of Liquid Fuel, of which the following is a specification.

In the operation of hydro-carbon engines, the difficulty arises of consuming the crude oil constituents of the fatty series which boil between 130° and a point not exceeding 400° C., and which give off particularly large amounts of heat calories in burning, completely and as rapidly as the low-boiling oils having boiling points below 130° C. The object of this invention is to render the high-boiling crude oil constituents suitable for use as fuel for hydro-carbon engines—explosion motors, for example—and in any of the carbureters now in general use for benzene. The new product which the invention proposes is characterized by the three following constituents:

1. At least one crude oil constituent of the fatty series, boiling between 130° and a point not exceeding 400° C.;  
 2. Hydro-carbons having a boiling point below 300° C. and of such a composition as will be obtained by the distillation of a tar; 30  
 3. Small additions of other light combustible substances, such as ketones, for example: acetone, aldehyde; or ethers or esters; or alcohols, for example: methyl alcohol; or mixtures thereof.

35 The improved product is obtained by preparing a mixture of at least one crude oil constituent of the fatty series boiling between 130° and a point not exceeding 400° C., hydro-carbons having a boiling point below 300° C. and of such a composition as may be obtained by distillation of a tar, and small additions of other light combustible substances.

45 The fatty series of crude oil constituents boiling between 130° and a point not exceeding 400° C., may be considered as including the hydro-carbons which are found in crude petroleum or which have their characteristics. Accordingly, a suitable petroleum oil can be used, or, for instance, the hydro-carbons obtained from the distillation of coal at low temperature, which are analogous to crude petroleum, or generator tar-oils. The combustible material may also 50 consist of crude oils of the fatty series other

than those having boiling points between the above-mentioned limits. For example, it can consist of petroleum hydro-carbons which distil at temperatures between 30° and 130° C. In this case, the whole fraction 60 distilling between 30° and 360° and up to 400° C. can be used for the preparation of the combustible. To the other hydro-carbons boiling below 300° C. and defined under the heading "2" above, belong those obtained, for example, by the distillation of coal tar, brown-coal tar, soft-coal tar, wood tar and the like, and those found in certain crude oils such as crude Borneo oil.

Example 1.—50 parts by weight of crude 70 petroleum distillates having a boiling point between 130° and up to but not exceeding 400° C., are mixed with 45 parts by weight of tar distillates, and about 5% of acetone (water free). A milky liquid is thereby obtained which gradually clears up when allowed to stand. The liquid may be filtered.

Example 2.—Crude East India oil (Borneo oil) which, in addition to crude oil constituents of the fatty series having a boiling point between 130° and the upper limit of 400° C., contains, as is well known, up to 40% of the hydro-carbons included in group 2, is mixed with 5% of acetone. The mixture may be filtered.

For the recovery of the above-mentioned hydro-carbons which boil below 300° C. and of such a composition as to be obtainable by the distillation of tar, the procedure is best carried out as follows:

Tar, obtained by coking coal, brown coal, etc., is once cleaned and distilled under pressure, either at from 75° to 130° or, if very high-powered motors are involved, then at from 75° to 150° or to 180° or to 210°. For 95 operating internal combustion engines, the tar can be distilled from 75° to 250°, or from 75° to 300°.

The new fuel is eminently suitable not only for explosion engines, but also for 100 Diesel and other motors. In comparison with benzene and other fuels, it possesses a higher efficiency, does not rust or soot, and is cheaper to manufacture. Moreover, it has the advantage that it can be mixed in suitable proportions with alcohol in any form.

I claim:

1. A fuel for combustion engines, containing at least one crude oil constituent belonging to the fatty series boiling between 110

130° and a point not exceeding 400° C.; acetone to a mixture of at least one crude hydro-carbons having a boiling point below 300° C., and of such a composition as will be obtained by the distillation of tar; and a small quantity of acetone.

2. The herein-described method of producing fuel for combustion engines, comprising the step of adding a small quantity of

oil constituent belonging to the fatty series <sup>10</sup> boiling between 130° and a point not exceeding 400° C. and hydro-carbons boiling below 300° C. and having such a composition as will be obtained by the distillation of tar.

In testimony whereof I affix my signature.

JACOB DOLFEN.